

Oct. 3, 1944.

C. C. SMITH

2,359,590

ELECTRICAL CONDUCTOR AND A METHOD OF MAKING IT

Filed Oct. 5, 1940



INVENTOR

C. C. SMITH

BY

E.S.R. Nowlan

ATTORNEY

## UNITED STATES PATENT OFFICE

2,359,590

ELECTRICAL CONDUCTOR AND A METHOD  
OF MAKING IT

Charles C. Smith, Cranford, N. J., assignor to  
Western Electric Company, Incorporated, New  
York, N. Y., a corporation of New York

Application October 5, 1940, Serial No. 359,878

4 Claims. (Cl. 154—2.25)

This invention relates to electrical conductors and a method of making them, and more particularly to insulated electrical wires and a method of making them.

For various uses, especially in the field of telephone apparatus, electrical conductors have long been insulated by being covered with wrappings of textile fiber threads served over the wire and subsequently coated with an additional outer layer or covering of material applied in liquid form and dried. An example of such insulated wire of particularly wide application in telephone apparatus has a core of copper wire which may be a single, solid strand or may consist of a plurality of small strands laid together in parallel relation or intertwined together or interbraided together. On this core are served, or sometimes knitted or braided, one or more coverings of silk threads; and one or more coverings of cotton thread are served, or sometimes knitted or braided, over the silk coverings. The covered wire is then passed through a bath of a liquid preparation of cellulose acetate or other suitable cellulose ester dissolved in a vehicle comprising acetone as the principal solvent agent. The solvent is then dried out, leaving a protective film or coating of cellulose acetate on and sometimes more or less impregnating the outer cotton covering. Insulated wires thus made are found to have eminently satisfactory electrical properties as well as mechanical strength and resistance to damage. Since the appearance of artificial silk in commerce, many attempts have been made to substitute artificial silk for real silk in the covering of wire as described. However, most of the artificial silk materials used in commercial threads comprise esters of cellulose, usually the acetate and sometimes the nitrate, as a principal component, and these are quickly soluble in acetone liquid and also absorb vapors of acetone more or less greedily and soften, melt or dissolve. Hence attempts to make such wires as above described with artificial silk replacing real silk in the inner coverings have not been satisfactory. The silk servings, if not wholly destroyed by liquid acetone soaking through the overlying cotton layers from the cellulose acetate in acetone baths, are softened, melted and coalesced more or less, or dissolved by vapors of acetone from the same source, especially during stoppages of the apparatus to repair breaks in the wire or to replace empty supply reels therein. Thus wires covered with artificial silk and with cotton over the silk and with cellulose acetate over the cotton, although highly desirable when the threads

of the artificial silk coverings keep their individual identity, because of high flexibility and excellent electrical and mechanical properties combined with materially lower cost, as compared with those in which real silk is used, have not been successfully manufactured heretofore.

An object of the present invention is to provide an insulated electrical wire having covering of cellulose acetate or the like and of artificial silk threads or the like material easily damaged by acetone or the like, separated by an intermediate covering of fibers of cotton or other material inert to the solvent action of acetone.

With the above and other objects in view, the invention may be embodied in an insulated electrical conductor wire comprising a conductive core, a covering thereon of fibrous material soluble in acetone or its vapors, a covering thereover of fibrous material inert to acetone and its vapors, and a coating thereon of amorphous cellulose ester material.

A further embodiment of the invention may present a method making such wire which comprises steps of serving, knitting or braiding a covering of threads of textile material soluble in acetone or its vapors on a wire, serving, knitting or braiding a covering of threads of textile material inert to acetone and its vapors over the said first named covering, extruding a coating of a thickly viscid preparation of cellulose ester softened in acetone over the second named covering and drying out the acetone.

Other objects and features of the invention will appear from the following detailed description of its embodiment in an insulated wire and a method of making insulated wire, taken in connection with the accompanying drawing, the single figure of which presents an enlarged diagrammatic view in side elevation of a piece of insulated wire constructed in accordance with the invention.

As herein disclosed and illustrated in the single figure on the drawing, a wire constructed in accordance with the invention may comprise a conductive core 10, a first covering 11 of artificial silk on the core, a second covering 12 of artificial silk over the first covering, a third covering 13 of cotton over the second covering, and an outer coating 14 of cellulose acetate over the third covering.

Each of the coverings 11, 12 and 13 consists essentially of textile threads served, knitted or braided in place by means of methods and apparatus too well known to require elucidation or illustration here. In the specific case illustrated

in the drawing, the covering 11 is served with a left hand pitch directly on the bare wire 10; the covering 12 is served with right hand twist directly on the covering 11; and the covering 13 is served with left hand twist directly on the covering 12. Each of these coverings is illustrated as served; but any one or two or all three may be knitted or braided if desired. In the actual case used as illustration here, the threads used to form each of the coverings 11 and 12 were of "Rayon," a commercial artificial silk consisting essentially of cellulose acetate; and the covering 13 was of cotton thread.

The coating 14 is of amorphous cellulose acetate. It is made by extruding over and drying on the covering 13 a coating of an extremely viscous preparation of cellulose acetate and other solids softened by being compounded with a solvent consisting essentially of acetone. To illustrate the nature of the raw coating material used, a suitable preparation will contain by weight 27% of cellulose acetate and 40% of acetone with 31% of other solids (plasticizers, fillers etc.) and 2% of other liquids. Another way of describing the essentials of this coating material is to say that it contains 72 ounces of cellulose acetate per gallon of acetone. The characterizing features of the material relevant to the present invention are the presence in material amount of acetone which is harmful, whether as liquid or as vapor, to "Rayon," and the high viscosity of the material as used. Measured under ordinary laboratory conditions, the viscosity of this material at 75° F. is about 25,000 poises, while at the extrusion temperature of about 105° F. it is about 18,000 poises. A suitable method and apparatus for extruding and drying the coating 14 are respectively disposed and claimed in applications Serial Nos. 209,396 and 295,024, filed respectively on May 21, 1938, and September 15, 1939, both by Edwin E. Newton et al. Application No. 295,024 has matured to Patent No. 2,260,830, dated Oct. 28, 1941.

A coating 14 of such material extruded over the covering 13 forms a tough, amorphous, seamless film entirely covering the covering 13 and more or less bonded into the superficial portion of the covering 13, as indicated at 15, by the extrusion pressure. Due to the volatility of acetone and the relatively small proportion of it present in the raw coating material, the acetone is evaporated immediately after the raw coated strand leaves the extruding means before enough acetone vapor, much less enough liquid acetone passes through the coating 13 to cause the threads to adhere together or even coalesce wholly and thereby damage the coverings 12 or 11.

Where attempts are made to effect the same result by passing the thread covered strand (10, 11, 12 and 13) through the liquid bath of cellulose acetate in acetone used in the case of wire covered with real silk and cotton, it is found that after drying, one or even both of the "Rayon" coverings 11 and 12 may have disappeared entirely, having been extracted by the acetone, or, at best, that their structure has disappeared entirely and they have become so diminished or irregular in thickness as to be worthless in practice. It is only where the cellulose acetate paste used is so low in acetone relatively to its content of cellulose acetate that its viscosity is upward of 7,000 poises at 75° F. that such coatings can be satisfactorily applied without damage to the "Rayon" or similar coverings 11 and 12 under the cotton covering 13. The solutions used for

coating real silk covered wire are a totally different thing in physical character. Typically they contain only two-fifths as much solids in proportion to solvent, and are sirupy, freely flowing liquids; whereas the materials herein disclosed are perhaps technically liquid, but are in consistency like very thick warm tar and cannot be used as a means for coating by dipping.

While the invention is herein illustratively disclosed as embodied in an insulated wire comprising a covering of mutually wholly independent cellulose acetate fibers and an outer coating of amorphous cellulose acetate separated by a covering of cotton fiber, and also as embodied in a method of making such wire which characteristically includes a step of extruding a very viscous preparation of cellulose acetate in acetone upon the cotton covering to form the amorphous coating, it will be clear that the invention is not so limited. An inner coating of cellulose nitrate is as subject to destruction by acetone liquid or vapor as cellulose acetate. So also the acetone ingredient might under some conditions be replaced by another such as toluol, xylol, or the like able to attack the material of the inner coverings 11 or 12. Furthermore, while the preferred material for the covering 13 is cotton on account of its mechanical properties, cheapness and satisfactory insulating qualities, this covering might be of wool or linen or other suitable fiber not susceptible of attack by the solvent used.

The embodiments particularly disclosed herein are illustrative and may be modified and departed from without departing from the spirit and scope of the invention as pointed out in and limited only by the appended claims.

What is claimed is:

1. The method of making insulated electrical conductor wire which comprises steps of forming on a wire a covering of insulating fibrous material susceptible of attack by the vapors as well as the liquid form of a specific solvent liquid, forming over the said covering a second covering of insulating fibrous material not susceptible of attack by the said solvent, and extruding upon the outer surface of the said second covering a coating of insulating material softened with an insufficient amount of the said solvent to allow even the vapors of the solvent to penetrate materially through the second covering to attack the first covering.
2. The method of making insulated electrical conductor wire which comprises steps of forming on a wire a covering of insulating fibrous cellulose ester susceptible of attack by the vapors as well as the liquid form of a specific solvent liquid, forming over the said covering a second covering of insulating fibrous cellulose not susceptible of attack by the said solvent, and extruding upon the outer surface of the said second covering a coating of insulating material softened with an insufficient amount of the said solvent to allow even the vapors of the solvent to penetrate materially through the second covering to attack the first covering.
3. The method of making insulated electrical conductor wire which comprises steps of forming on a wire a covering of threads of cellulose acetate, forming over the said covering a covering of cotton threads, and extruding upon the outer surface of the cotton thread covering a coating of thickly viscous material of viscosity not less than 7,000 poises at 75° F. and containing cellulose acetate and acetone as its principal ingredients, whereby to leave the cellulose acetate

threads substantially unaffected by even the vapors of the acetone.

4. The method of making insulated electrical conductor wire which comprises steps of forming on a wire a covering of threads of cellulose acetate, forming over the said covering a covering of cotton threads, and extruding upon the outer surface of the cotton thread covering a coating

of thickly viscid material of viscosity of the order of 25,000 poises at 75° F. and containing cellulose acetate and acetone as its principal ingredients, whereby to leave the cellulose acetate threads substantially unaffected by even the vapors of the acetone.

CHARLES C. SMITH.